

# UNITED STATES PATENT OFFICE.

THOMAS B. PARKISON, OF MUNCIE, INDIANA, ASSIGNOR TO UNION FIBRE COMPANY,  
OF WINONA, MINNESOTA, A CORPORATION OF MINNESOTA.

## NON-CONDUCTING MATERIAL AND PROCESS OF MAKING SAME.

1,078,307.

Specification of Letters Patent. Patented Nov. 11, 1913.

No Drawing. Continuation of application Serial No. 461,942, filed November 10, 1908. This application filed July 31, 1909. Serial No. 510,670.

*To all whom it may concern:*

Be it known that I, THOMAS B. PARKISON, a citizen of the United States, residing at Muncie, in the county of Delaware and 5 State of Indiana, have invented a new and useful Non-Conducting Material and Process of Making Same, of which the following is a specification.

This invention relates to non-conducting 10 insulating material adapted for lining houses, cold storage chambers, refrigerating cars, or for covering steam pipes and the like, for preventing the conduction of sound, heat or cold and to the process of making 15 the same; and the principal object of the invention is the production of an improved "lith" which is an insulating material composed of mineral wool and a suitable binder, or mineral wool and degummed flax fiber, 20 compounded according to the methods set forth in the United States patents granted to George Kelly, No. 665,229 of Jan. 1st, 1901, and No. 811,227, of January 30, 1906, the present invention residing in the manu- 25 facture of an insulating material possessing all the desirable qualities of the commercial "lith", while having the further property of resisting moisture and, in some instances, resisting fire.

30 In carrying out the invention, mineral wool constitutes the chief ingredient because of its superior insulating qualities, and this is preferably treated after the process disclosed in my Patent Number 945,583, dated January 4, 1910, by which the individual 35 filaments or fibers of the mineral wool are coated with a volatile oil during the process of forming the fibers from the molten slag, by directing petroleum into the blast that 40 produces the filamentary form, with the result that the petroleum is converted into smoke, which penetrates the mass of moving fibers and coats them with the hydrocarbon, so that the coating aids, to a great extent, 45 in waterproofing the material. The mineral wool, thus prepared, is in the simplest form of the material, mixed with a suitable binder, such as paper stock, or any glutinous substance which will not impair the insulating 50 qualities of the product. In other forms of the material, the mineral wool is mixed with either flax fiber or asbestos fiber, depending wholly upon the character of the product desired. A waterproofing

liquid is employed, consisting of either 55 bitumen or asphaltum heated until liquefied and mixed with a relatively crude carbonaceous oil, such as petroleum. The materials made use of are commingled with the said liquid, and thereafter the product is molded 60 or shaped in the form of slabs, tiles or boards, and then dried. The waterproofing liquid readily combines with the coating on the mineral wool, so that the resulting product will have a great repelling power to 65 moisture and yet, at the same time, the insulating qualities well known to exist in commercial "lith" are retained. The binder whereby the fibers of the mineral wool are held together as a self-sustaining mass, may 70 be some vegetable or other glue when paper stock is not used. When paper stock is employed the sizing used in the production of the paper will serve as a binder for the mineral wool, and the paper fiber materially 75 contributes to give a body to the waterproof material.

When it is desired to produce waterproof 80 boards, slabs and the like, having considerable tensile strength, some fibrous material is added to the composition. Degummed flax fiber is commonly used for this purpose when merely a waterproof "lith" is desired; or, by substituting asbestos for the flax fiber, 85 a fireproof quality is imparted to the material though the tensile strength is lessened. When asbestos is employed, the binder will be preferably some vegetable or other glutinous substance and the paper stock can be dispensed with, and is made optional. The 90 degummed flax fiber will be prepared under the process described in the Kelly Patent, No. 665,229.

To explain more in detail the making of 95 this improved form of "lith", the ingredients which may be used are as follows: Fifty pounds of asphaltum, nine gallons of crude petroleum, two hundred pounds of paper stock or pulp, two hundred and fifty pounds of flax shive or degummed flax fiber, 100 nine hundred pounds of mineral wool coated with volatile oil, and in addition an indefinite but small quantity of either mineral wool or sawdust from "lith" to thicken the waterproofing liquid. In preparing the 105 compound the asphaltum is liquefied by heat and the crude petroleum added thereto for forming the waterproofing liquid, and to

this liquid is supplied for thickening purposes mineral wool, or sawdust made from cutting blocks of waterproof "lith" produced according to the present method, and 5 in such quantity that the resulting waterproofing liquid will have the consistency of apple butter. In the meantime, the paper stock, if such is used, is put into a beater and beaten to a pulp and the flax shive then 10 added to the beater, and after these two are thoroughly commingled, the waterproofing liquid as above set forth is added. A few revolutions of the beater are sufficient 15 to mix the waterproofing liquid with the paper pulp and shives. Following this, the nine hundred pounds of mineral wool are added and mixed but not beaten in with the mixture already in the beater. After the ingredients are thoroughly mixed, the contents of the beater are emptied into the 20 molds and finally baked.

Of course, when a waterproof and fireproof product is desired, the flax fiber is dispensed with and asbestos fiber substituted, and in this latter case, some suitable 25 glutinous binder is employed instead of paper pulp.

The waterproof qualities in the product are obtained from two sources: first, by the 30 waterproofing of the mineral wool particles under the Parkison process, as described and claimed in the aforesaid patent; and second, by the addition of the waterproofing liquid in the commingling of the various materials.

I consider that I am the first to waterproof mineral wool by applying crude petroleum to the particles or filaments thereof during the process of manufacturing the 40 wool. This wool may be used alone as an insulator, but in practice is associated with either paper stock or other glutinous substance, or with asbestos or flax fiber. While reliance could be made upon the initial 45 treatment of the wool as a waterproofing thereof, it is the preferable practice to employ the waterproofing liquid, and I regard its use as an important step in the production of a commercial product.

50 This application is a continuation of my former application No. 461,942, filed November 10, 1908.

Having thus described the invention, what I claim as new, and desire to secure by Letters-Patent, is:—

1. The method of producing a waterproof insulating composition consisting of subjecting mineral wool to the action of smoke of burning petroleum during the process of manufacturing the wool, and combining with the wool so treated a binder, and a fiber of greater tensile strength than mineral wool.

60 2. The method of producing a waterproof insulating composition consisting of subject-

ing mineral wool to the action of smoke of 65 burning petroleum during the process of manufacturing the wool, and combining with the wool so treated a binder, and a waterproofing liquid.

3. The method of producing a waterproof 70 insulating composition consisting of subjecting mineral wool to the action of smoke of burning petroleum during the process of manufacturing the wool, and combining with the wool so treated a binder, a fiber of 75 greater tensile strength than mineral wool, and a waterproofing liquid.

4. The method of producing an insulating composition which consists in coating mineral wool with a hydrocarbon during the 80 process of manufacture by subjecting the same to the action of smoke of burning petroleum, then commingling therewith flax fiber and a binder, and shaping and drying the composition.

85 5. The method of producing a waterproof composition, which consists in coating with a hydrocarbon oil mineral wool fiber during the process of manufacturing the latter by subjecting the same to the action of smoke 90 of burning petroleum, combining therewith another fiber and paper pulp, and finally molding the commingled mass and drying the same.

6. The method of producing a waterproof 95 insulating composition, which consists in treating mineral wool by bringing it into contact with smoke from the combustion of petroleum, and then commingling the mineral wool so treated with a liquid hydrocarbonaceous material, and finally shaping and 100 drying the resulting product.

7. The method of producing a waterproof insulating composition, which consists in treating mineral wool by bringing it into 105 contact with smoke from the combustion of petroleum, and then commingling the mineral wool so treated with a liquid hydrocarbonaceous material and a fiber of greater tensile strength from the mineral wool.

110 8. An insulating composition including mineral wool, the individual fibers of which have been coated during the process of manufacture with the smoke of burning petroleum, combined with a waterproofing 115 liquid.

9. An insulating composition composed of mineral wool, the fibers of which have been subjected to the action of smoke of burning petroleum during the process of manufacture, combined with a waterproofing liquid, and a flax fiber.

120 10. An insulating composition including mineral wool the individual fibers of which are coated during the process of manufacture 125 with smoke from burning petroleum.

11. An insulating composition composed of a binder, a mixture of liquid asphaltum

and petroleum, and mineral wool, the fibers of which have been previously coated with hydrocarbonaceous material, the mass so formed being molded and dried.

- 5 12. An insulating composition composed of the following ingredients in the following proportions:—fifty pounds of asphaltum, nine gallons of crude petroleum, two hundred and fifty pounds of flax shives, and
- 10 nine hundred pounds of mineral wool which

has been previously treated to coat it with hydrocarbonaceous material, and a binder.

In testimony, that I claim the foregoing as my own, I have hereto affixed my signature in the presence of two witnesses.

THOMAS B. PARKISON.

Witnesses:

WILLIAM OVERMIRE,  
LULA ADAMS.